

United States Patent [19]  
Strepparola et al.



US005190681A

[11] Patent Number: 5,190,681  
[45] Date of Patent: Mar. 2, 1993

[54] ANTIRUST ADDITIVES FOR LUBRICANTS  
OR GREASES BASED ON  
PERFLUOROPOLYETHERS

[75] Inventors: Ezio Strepparola, Treviglio; Piero  
Gavezotti; Costante Corti, both of  
Milan, all of Italy

[73] Assignee: Ausimont S.r.l., Milan, Italy

[21] Appl. No.: 715,692

[22] Filed: Jun. 17, 1991

Related U.S. Application Data

[63] Continuation of Ser. No. 335,227, Apr. 10, 1989, aban-  
doned.

[30] Foreign Application Priority Data

Apr. 13, 1988 [IT] Italy ..... 20183 A/88

[51] Int. Cl.<sup>5</sup> ..... C10M 147/04

[52] U.S. Cl. ..... 252/51.5 R; 252/54;  
252/58; 252/51; 558/447; 558/461

[58] Field of Search ..... 252/51.5 R, 54, 475;  
558/447, 461

[56] References Cited

U.S. PATENT DOCUMENTS

3,293,306 12/1966 LeBleu et al. ..... 252/54  
3,367,868 2/1968 Skehan ..... 252/51.5 R  
3,505,411 4/1970 Rice ..... 558/447  
3,536,624 10/1970 Christian et al. ..... 252/54

3,665,041 5/1972 Sianesi et al. ..... 252/54  
3,697,564 10/1972 Anello et al. ..... 558/447  
3,847,978 11/1974 Sianesi et al. ..... 558/447  
4,011,255 3/1977 Tamborski ..... 558/447  
4,058,469 11/1977 Hoke ..... 252/51.5 R  
4,085,137 4/1978 Mitsch et al. ..... 260/561 HL  
4,113,772 9/1978 Lagow et al. ..... 562/583  
4,132,660 1/1979 Christian et al. ..... 252/51.5 R  
4,194,983 3/1980 Paciorek et al. ..... 252/49.9  
4,404,377 9/1983 Seale et al. ..... 544/87  
4,647,413 3/1987 Savu ..... 558/447  
4,757,145 7/1988 Caporiccio et al. ..... 252/51.5 R

Primary Examiner—Ellen McAvoy

Attorney, Agent, or Firm—Morgan & Finnegan

[57] ABSTRACT

An antirust additive for lubricants based on perfluoropolyethers, comprising one of the fluoropolyether compounds having functionalized end groups selected from —CN, —CH<sub>2</sub>NR<sub>1</sub>R<sub>2</sub> and



and in particular a combination of these with small amounts of a fluoropolyether with acid end groups.

5 Claims, No Drawings



-continued



where at least one of end groups T and T' is selected from

- (a) —CFX—CN;  
 (b) —CFX—CH<sub>2</sub>—NR<sub>1</sub>R<sub>2</sub>, where R<sub>1</sub> and R<sub>2</sub> are the same as defined above;  
 (c)



where A and R are the same as defined hereinbefore; where X in (a), (b) and (c) is F or CF<sub>3</sub>;

the other end group T or T' may be a perfluoroalkyl radical with 1 to 3 carbon atoms;

indexes g, h, m, n, k, j, p, q, s, t, r, u, v, z, x, y are integers selected in such manner that the average molecular weight of the polyoxyfluoroalkylene chain ranges from 600 to 6,000, and preferably from 2,000 to 4,000 for difunctional compounds and from 1,000 to 2,000 for monofunctional compounds;

R<sub>f</sub> is a fluoroalkylene radical;

R'f is a fluoroalkyl radical;

the oxyfluoroalkylene units being statistically distributed along the chain.

Generally, the additives of this invention exhibit a solubility in the PFPE lubricant of at least 1% by weight referred to the lubricant. The amount of the above antirust fluoropolyether additives preferably ranges from 1% to 5% by weight based on the total amount of lubricant, and more preferably from 2% to 4%.

If the lubricant in which the antirust additive is utilized is a grease based on perfluoropolyether, this may be prepared as is described in European patent application No. 92,825. In particular, such grease may be formulated by suspending polytetrafluoroethylene particles, having for example a spherical morphology and being composed of aggregates having sizes from 1 to 200 microns, in a perfluoropolyether liquid such as Fomblin®Y or Fomblin®Z.

The compounds having end groups of the types (b) and (c) indicated above may also be utilized as such in consideration of their intrinsic lubricating properties.

Furthermore, it has been discovered that the additives having the end groups (a), (b) and (c) indicated above may be used in combination with small amounts of fluoropolyether compounds having the same chain structure as the compounds belonging to classes I

through XI and one or two end groups —CFX—COOH, where X is F or CF<sub>3</sub>, generally in an amount ranging from 1/30 to 1/20 by weight of the additive characterized by end groups (a), (b) or (c).

5 The precursors having a fluoropolyether structure of the additives of the present invention are preparable as follows:

those of class (I) according to the processes described in U.S. Pat. No. 3,242,218;

10 those of class (II) according to U.S. Pat. No. 3,665,041;

those of classes (III) and (IV) according to published European patent application EP 148,482;

those of class (V) according to U.S. Pat. No. 4,523,039;

those of class (VI) according to published European patent application EP 151,877;

those of class (VII) according to U.S. Pat. No. 3,665,041;

those of class (VIII) according to U.S. Pat. No. 3,250,808;

those of class (IX) according to EP 148,482;

those of class (X) according to the processes described in International patent application WO87/00538; and

25 those of class (XI) according to the processes described in International patent application WO87/02992.

The above end groups may be obtained by the method described in U.S. Pat. No. 3,010,874. In particular, the introduction of the end groups of type (a) is obtained starting from the corresponding derivatives with ester end groups —CFX—COOR<sub>3</sub> (R<sub>3</sub>=CH<sub>3</sub>, C<sub>2</sub>H<sub>5</sub>, C<sub>6</sub>H<sub>5</sub>) by treatment with anhydrous ammonia, preferably in a solvent such as, for example, ethyl ether, methanol, or 1,1,2-trichlorotrifluoroethane, and subsequent treatment of the resulting amide with P<sub>2</sub>O<sub>5</sub>.

The introduction of end groups of types (b) and (c) is obtained by reacting the ester compounds indicated above, respectively, with an amine NHR<sub>1</sub>R<sub>2</sub> or with an amine having the formula:



50 to provide the respective amides, and by subsequent reduction with hydrides.

In the case of classes (II), (III), (V), (VII), (VIII), (IX), and (X) in which the starting perfluoropolymers have only one functional end group, it is possible to 55 achieve the corresponding bifunctionalized product by means of the process described in European patent application EP 224,201.

The antirust properties of the added lubricants according to the present invention have been evaluated 60 by means of the following tests:

#### Antirust test in the fog chamber

#### Method ASTM D.1748, modified

Object: Determination of the antirust properties of 65 oils on metals under conditions of high humidity.

Summary of the method: carbon steel plates (C15) (UNI) - superficially treated as is described hereinafter -- were dipped into the oil, allowed to drip and hung in

a fog chamber at 50° C. and 100% of relative humidity, for a pre-determined number of hours. The oil passes or does not pass the test depending upon the number of rust stains which are visible on the surface of the plates.

Apparatus: The fog chamber consists of a compressed-air-actuated sprayer ( $P=3$  atm.), connected with a water reserve and such as to saturate the environment with humidity; the temperature check was adjusted at 50° C. (see ASTM B.117, 287, 368).

Test conditions: The tests described hereinafter were carried out using partially demineralized water ( $\text{pH}=5.5-7.5$ ) for periods of time as follows:

- (1) the plates were hung and allowed to drip for 16 hours;
- (2) they were then placed into a fog chamber, which was kept in operation during 8 hours;
- (3) the fog chamber was kept out of operation during 12 hours;
- (4) the fog chamber was turned on again and kept in operation during 8 hours.

Then the evaluation was carried out.

Preparation of the steel plates: The steel plates were cleaned and degreased by means of a cloth saturated with Delifrene 113 (trichlorotrifluoroethane); the surface was polished by means of rubbing papers (400 meshes and 600''), then they were washed with water and dried. The steel plates utilized had the following dimensions:  $50 \times 100 \times 2$  mm. (Note: polythene gauntlets must be used to handle the plates.)

Evaluation of the tests: (By analogy with method DIN 51802 (EMCOR) for bearings).

The results of the tests are expressed according to the following classifications:

- (0) no traces of rust are observed;
- (1) very few corrosion points having a diameter below 1 mm;

- (2) 30% of the surface is covered by little stains having a diameter below 2 mm;
- (3) 60% of the surface is covered by little stains having a diameter below 3 mm;
- (4) 100% of the surface is covered by large stains having a diameter of 4-5 mm, but the polished surface is visible in some points;
- (5) 100% of the surface is covered by large stains; the underlying surface is not visible.

In the evaluation, the rust stains appearing in the area up to 0.5 mm from the edges are not taken into consideration. If the evaluation is (0), the test has been met.

In the evaluation, two figures are indicated: the first figure refers to the state of the exposed face; the second figure refers to the non-exposed face (with respect to the sprayer).

## EXAMPLES

The following examples are given to illustrate the present invention, without however being a limitation thereof.

### EXAMPLE 1

Lubricants consisting of perfluoropolyether having perfluoroalkyl end groups Fomblin® Y25, characterized by a viscosity of 250 cSt at 20° C., additioned with the compounds indicated in the following Table 1, were subjected to the accelerated corrosion test in a fog chamber according to the method described above.

Table 1 shows the weight % of the additive with respect to the perfluoropolyether and the results of the corrosion test, expressed by the indices reported above in the description of the method.

TABLE 1

| Additive                                                                                                                                                                                                                                                        | Tests on Fomblin® Y25 |          |        |
|-----------------------------------------------------------------------------------------------------------------------------------------------------------------------------------------------------------------------------------------------------------------|-----------------------|----------|--------|
|                                                                                                                                                                                                                                                                 | M.W.                  | Weight % | Result |
| (a) $\text{NC}-\text{CF}_2\text{O}(\text{CF}_2\text{CF}_2\text{O})_m(\text{CF}_2\text{O})_n-\text{CF}_2\text{CN}$<br>$\text{HOOC}-\text{CF}_2\text{O}(\text{CF}_2\text{CF}_2\text{O})_m(\text{CF}_2\text{O})_n-\text{CF}_2\text{COOH}$                          | 2000                  | 2        | 0-0    |
|                                                                                                                                                                                                                                                                 | 2000                  | 0.1      |        |
| (b) $\text{NC}-\text{CF}_2\text{O}(\text{CF}_2\text{CF}_2\text{O})_m(\text{CF}_2\text{O})_n-\text{CF}_2\text{CN}$<br>$\text{HOOC}-\text{CF}_2\text{O}(\text{CF}_2\text{CF}_2\text{O})_m(\text{CF}_2\text{O})_n-\text{CF}_2\text{COOH}$                          | 2000                  | 3        | 0-0    |
|                                                                                                                                                                                                                                                                 | 2000                  | 0.1      |        |
| (c) $\text{NC}-\text{CF}_2\text{O}(\text{CF}_2\text{CF}_2\text{O})_m(\text{CF}_2\text{O})_n-\text{CF}_2\text{CN}$                                                                                                                                               | 2000                  | 2        | 0-0    |
| (d) $\text{CF}_3\text{O} \left( \begin{array}{c} \text{CF}_2\text{CFO} \\   \\ \text{CF}_3 \end{array} \right)_m (\text{CF}_2\text{O})_n-\text{CF}_2-\text{CH}_2\text{N} \begin{array}{c} \text{O} \\ \text{C} \\ \text{C} \\ \text{C} \\ \text{O} \end{array}$ | 1000                  | 2        | 0-0    |
|                                                                                                                                                                                                                                                                 |                       |          |        |
| (e) $\text{CF}_3\text{O} \left( \begin{array}{c} \text{CF}_2\text{CFO} \\   \\ \text{CF}_3 \end{array} \right)_m (\text{CF}_2\text{O})_n-\text{CF}_2-\text{CH}_2\text{N} \begin{array}{c} \text{O} \\ \text{C} \\ \text{C} \\ \text{C} \\ \text{O} \end{array}$ | 1000                  | 5        | 0-0    |
|                                                                                                                                                                                                                                                                 |                       |          |        |
| (f) $\text{CF}_3\text{O} \left( \begin{array}{c} \text{CF}_2\text{CFO} \\   \\ \text{CF}_3 \end{array} \right)_m (\text{CF}_2\text{O})_n-\text{CF}_2\text{CH}_2\text{NH}_2$                                                                                     | 900                   | 2        | 1-0    |
|                                                                                                                                                                                                                                                                 |                       |          |        |
| (g) $\text{CF}_3\text{O} \left( \begin{array}{c} \text{CF}_2\text{CFO} \\   \\ \text{CF}_3 \end{array} \right)_m (\text{CF}_2\text{O})_n-\text{CF}_2\text{CH}_2\text{NH}_2$                                                                                     | 900                   | 4        | 0-0    |
|                                                                                                                                                                                                                                                                 |                       |          |        |

## EXAMPLE 1A

Example 1 was repeated using, as a lubricant, non-additived perfluoropolyether Fomblin® Y25. The result was a complete corrosion of the plate: 5-5.

## EXAMPLE 1B

Example 1 was repeated using, as a lubricant, Fomblin® Y25 additived with the mixture:



M.W.=2,000; 2%

and



M.W.=2,000; 0.1%

soluble in the perfluoropolyether.

The result of the test was 3-2.

## EXAMPLE 2

Lubricants consisting of perfluoropolyether having perfluoroalkyl end groups Fomblin® Z25, characterized by a viscosity of 250 cSt at 20° C., additived with the compounds reported in the following Table 2, were subjected to the accelerated corrosion test as in Example 1.

Table 2 shows the results of the tests.

TABLE 2

| Additive | Tests on Fomblin® Z25                                                                                                     |     | M.W. | Weight % | Result |
|----------|---------------------------------------------------------------------------------------------------------------------------|-----|------|----------|--------|
|          | (a)                                                                                                                       | (b) |      |          |        |
| (a)      | $\text{NC}-\text{CF}_2\text{O}(\text{CF}_2\text{CF}_2\text{O})_m(\text{C}-\text{F}_2\text{O})_n-\text{CF}_2\text{CN}$     |     | 2000 | 2        | 0-0    |
|          | $\text{HOOC}-\text{CF}_2\text{O}(\text{CF}_2\text{CF}_2\text{O})_m(\text{C}-\text{F}_2\text{O})_n-\text{CF}_2\text{COOH}$ |     | 2000 | 0.1      |        |
| (b)      | $\text{NC}-\text{CF}_2\text{O}(\text{CF}_2\text{CF}_2\text{O})_m(\text{C}-\text{F}_2\text{O})_n-\text{CF}_2\text{CN}$     |     | 2000 | 3        | 0-0    |
|          | $\text{HOOC}-\text{CF}_2\text{O}(\text{CF}_2\text{CF}_2\text{O})_m(\text{C}-\text{F}_2\text{O})_n-\text{CF}_2\text{COOH}$ |     | 2000 | 0.1      |        |

## EXAMPLE 2A

Example 2 was repeated using, as a lubricant, non-additived perfluoropolyether Fomblin® Z25. The result was a complete corrosion of the plate: 5-5.

## EXAMPLE 2B

Example 2 was repeated using, as a lubricant, Fomblin® Z25 additived with the mixture:



The result of the test was a rather good anticorrosive power (2-0), but the additive was insoluble in this type of perfluoropolyether.

## EXAMPLE 3

Subjected to the accelerated corrosion test as in Example 1 were the lubricants consisting of perfluoropolyether having perfluoroalkyl end groups Fomblin® YR 140/13, characterized by a viscosity of 1,400 cSt at 20° C., additived with the mixture:



5 The result of the corrosion test was 0-0.

## EXAMPLE 3A

10 Example 3 was repeated using, as a lubricant, perfluoropolyether Fomblin® YR 140/13 without additive. The result was a complete corrosion of the plate: 5-5.

## EXAMPLE 3B

15 Example 3 was repeated using, as a lubricant, Fomblin® YR 140/13 additived with the mixture:



20 M.W.=2,000, 2%

and



M.W.=2,000, 0.1%.

25 The result of the test was a rather good anticorrosive power (1-0), but the additive was insoluble in this type of perfluoropolyether.

30 Although the invention has been described in con-

junction with specific embodiments, it is evident that many alternatives and variations will be apparent to those skilled in the art in light of the foregoing description. Accordingly, the invention is intended to embrace all of the alternatives and variations that fall within the spirit and scope of the appended claims. The above references are hereby incorporated by reference.

35 What is claimed is:

50 1. Antirust additives for greases and lubricating oils

based on perfluoropolyethers, consisting of fluoropolyether compounds having at least one of the following repeating units:



-continued



a fluoroalkylene radical, and having at least one end group of formula:

—CFX—CN;

where X is F or CH<sub>3</sub>; and the other radical may be a perfluoroalkyl radical having 1 to 3 carbon atoms.

2. Antitrust additives for greases and lubricating oils based on perfluoropolyethers, comprising at least one of the following fluoropolyether compounds:



(I)

20



(II)



(III)

25



(IV)



(V)



(VI)



(VII)

30

where R' is a fluoroalkylene radical, and having at least one end group of formula: —CFX—CN; where X is F or CH<sub>3</sub>; and the other radical may be a perfluoroalkyl radical having 1 to 3 carbon atoms.



(VIII)

35

4. The greases and lubricating oils of claim 3, wherein the additives are in an amount ranging from 2 to 4% by weight calculated on the total amount of grease or lubricating oil.



(IX)

40

5. Greases and lubricating oils having antirust properties, based on perfluoropolyethers comprising the additives of claim 1 in combination with small amounts of fluoropolyether compounds having the same chain structure of said additives and one or two end groups —CFX—COOH, where X is F or CF<sub>3</sub>, in an amount ranging from 1/30 to 1/20 by weight of the additive of claim 1.

\* \* \* \* \*

where at least one of the end groups T and T' is of the formula:

—CFX—CN;